

# UNITED STATES PATENT OFFICE.

HERMANN G. C. THOFEHRN, OF NEW YORK, N. Y., ASSIGNOR TO LIGHT METALS CO.,  
OF ELIZABETH, NEW JERSEY.

## METHOD OF MAKING ALLOYS.

1,310,310.

Specification of Letters Patent. Patented July 15, 1919.

No Drawing.

Application filed December 15, 1917. Serial No. 207,312.

*To all whom it may concern:*

Be it known that I, HERMANN G. C. THOFEHRN, a citizen of the United States, and a resident of New York, in the county of New York and State of New York, have invented certain new and useful Improvements in Methods of Making Alloys; and I do hereby declare the following to be a full, clear, and exact description of the invention, such as will enable others skilled in the art to which it appertains to make and use the same.

This invention relates to improvements in the method of making alloys and more particularly to an improved method of making an alloy of aluminum, magnesium and uranium,—the object of the invention being to produce an alloy having great tensile strength, and which shall, at the same time be very light in weight.

With this object in view, the invention consists in certain novel steps in the method of making an alloy of the character specified, as hereinafter set forth and pointed out in the claims.

In carrying out the method for the production of the alloy, I first place in a suitable crucible or container a quantity of uranium oxid sufficient to provide in the finished alloy a uranium content of from 0.01 to 0.3 per cent., and apply heat to raise the temperature of the said uranium oxid to a bright red heat. I then introduce aluminum in the proportion of from 94 to 98 per cent. and when the mass has become molten, I add magnesium in the proportion of from 2 to 6 per cent. As these molten metals react upon the uranium oxid, the latter will be reduced to metal which is dissolved throughout the whole mass.

In order to avoid the metal retaining gases which would make it porous, I agitate the molten mass with the use of an iron rod having a disk of iron on one end. With the use of this tool, I perform a pumping action in the molten mass, agitating the same gently and causing the disk or headed end of the tool to remain under the surface of the mass to avoid splashing. Such gentle agitation will cause gases which

may be contained in the molten metal to escape, and thus a good sound casting may be obtained.

By means of my improved process, I obtain an alloy which is of exceedingly light weight but having great tensile strength and toughness and which is eminently suitable in the manufacture of structural work where a maximum of such qualities is an important consideration.

Having fully described my invention, what I claim as new and desire to secure by Letters Patent, is:

1. The herein described method, consisting in raising the temperature of uranium oxid to a bright red heat in a container, adding to said uranium oxid, aluminum and maintaining the temperature sufficiently high to render the aluminum molten, and then adding magnesium, and causing reactions which will reduce the uranium oxid to metal dissolved throughout the entire mass.

2. The herein described method consisting in heating uranium oxid to a bright red heat in a container, adding aluminum to said uranium oxid, maintaining sufficient heat to render the aluminum molten, then adding magnesium, and finally agitating the molten mass by a pumping action therein to expel any gases which it may contain.

3. The herein described method consisting in first raising to a bright red heat the temperature of uranium oxid corresponding in quantity to from 0.01 to 0.3 per cent. of the uranium content of the finished product; then adding aluminum in the proportion of from 94 to 98 per cent.; rendering the aluminum molten, and then adding to the molten mass, magnesium in the proportion of from 2 to 6 per cent.

In testimony whereof, I have signed this specification in the presence of two subscribing witnesses.

HERMANN G. C. THOFEHRN.

Witnesses:

DONALD H. McLEAN,  
VIVIAN L. ADELBERG.